

## UNITED STATES PATENT OFFICE

2,018,965

## CLEAN-UP AGENT

John D. McQuade, Lakewood, Ohio, assignor to  
Kemet Laboratories Company, Inc., a corpora-  
tion of New York

No Drawing. Application November 10, 1933,  
Serial No. 697,545

7 Claims. (Cl. 250—27.5)

The invention relates to clean-up agents for use in producing high vacuums, referring more specifically to clean-up agents comprising compacted comminuted metals and alloys.

- 5 To improve the vacuums of such high vacuum devices as thermionic valves, it is customary to vaporize a highly reactive material within the imperfectly evacuated device, whereby gases are adsorbed by or reacted with the active material.
- 10 This active material is commonly in the form of a "getter" tablet, lozenge, or pill. A frequently used method of vaporizing the clean-up agent is to mount the tablet on a tab, strip, or cup of metal within the device to be evacuated, and to 15 heat the tab and clean-up agent by inductive electric heating to the vaporizing temperature of the active material. The vaporizing operation is commonly termed "flashing".
- 15 All of the metals and alloys commonly used for getters, for example, barium, magnesium, sodium, barium-magnesium alloy, barium-strontium-magnesium alloy, barium-aluminum alloy, barium-silicon, mischmetal, and the like, are substantially silver-colored materials.
- 20 Similarly, all of the metals commonly used as supporting tabs or cups for the getters, for example, nickel and iron, are also substantially silver-colored materials.

25 As a result, partly of the similarity in the color of the getters and supporting tabs, and partly of the diminutive size of the usual getter tablet, careful inspection is required to ascertain whether a given getter and tab assembly actually contains a getter tablet. It is not at all an un- 30 common occurrence that the getter tablet is missing from an assembly placed in an otherwise perfect electronic device during manufacture of the latter, with the result that the electronic device must be scrapped. A more conspicuous 35 getter tablet would avoid most of such mishaps.

40 It is an object of the present invention to provide a getter tablet or pill, of the type above described, having a distinct color which renders the tablet conspicuous against a silver-colored background.

45 It is a further object of the invention to provide a getter tablet or pill comprising compacted comminuted metal more firmly coherent than the getters previously known.

50 A further object is to provide a getter tablet having improved stability in air.

55 These and other objects are attained in the present invention which provides a getter comprising comminuted active getter material and comminuted copper pressed into the form of a

tablet, pill, or lozenge. The copper, which is preferably intimately mixed with the active getter material, serves as an excellent bonding material, imparts a distinct reddish color, and improves the air stability of the getter without markedly influencing its effectiveness as a clean-up agent.

5 The active getter material suitably includes one or more of the following: an alkali metal, an alkaline earth metal; a rare earth metal; 10 mischmetal; an alloy or compound of one or more of these metals with aluminum, beryllium, magnesium, nickel, or silicon. An alloy containing at least about 15% of the alkali metal, alkaline earth metal, or rare earth metal, is suitable. An alloy comprising barium and magnesium, or barium, strontium, and magnesium, is preferred.

15 The copper may be of commercial purity, but is preferably relatively free from gases. Heating 20 the copper powder in a vacuum will yield a suitably gas-free material. Obviously, certain reddish or yellow brasses and bronzes may be substituted for the copper; but pure copper is preferred. Any sufficiently comminuted form is 25 suitable, for example, mechanically powdered copper, chemically precipitated copper, or electrolytically deposited finely dendritic copper.

20 The getter material may be mounted on the supporting tab or cup by forming the powdered 30 getter material into a tablet and pressing the tablet into a depression (which may or may not be preformed) in the tab or cup; or by pressing the loose getter material in place within a pre- 35 formed depression in the tab or cup; or by forming the tablet and the depression in one press- 40 ing operation. Alternatively, the getter material may be formed into a tablet or pill and supported on a tab, or in a cup, by a screen or other suit- able known holding means.

45 I have found by experiment that the clean-up agent of the invention preferably comprises about 50% to 75% of active material, such as barium-magnesium alloy, and about 25% to 50% of copper. Clean-up material having this com- 45 position has been pressed into depressions in nickel strips to form complete getter assemblies. The getter tablets contrasted sharply in color with the nickel strips, and the tablets were more firmly coherent, and more stable in air, than 50 similar tablets containing no copper.

55 I have also observed that the getter tablets of the invention, being inherently more coherent, are more easily fabricated than copper-free tablets, and may be fabricated in shapes and 55

sizes heretofore considered impossible or impractical to manufacture.

I claim:

1. A clean-up agent comprising a mixture of 5 comminuted copper and comminuted silver-colored active clean-up material, the copper forming about 25% to 50% of the mixture, the copper being physically separable from the active material and being present in sufficient amount to impart a reddish color to the clean-up agent.
- 10 2. A clean-up agent comprising an intimate mixture of comminuted copper and comminuted active material chosen from the group consisting of the alkali metals, the alkaline earth metals, the rare earth metals, and alloys thereof containing at least about 15% of the said metals; the copper forming about 25% to 50% of the mixture; the copper being physically separable from the active material and being present in 15 sufficient amount to impart a reddish color to the clean-up agent.
- 15 3. A clean-up agent comprising about 25% to 50% copper, the balance an alloy of barium, strontium, and magnesium; the copper being physically separable from the said alloy and being present in sufficient amount to impart a reddish color to the clean-up agent.
- 20 4. A getter assembly comprising a thin piece of substantially silver-colored metal provided with a circumscribed depression and firmly secured in the depression a reddish-colored clean-up agent containing about 25% to 50% copper up agent.
- 25
- 30

and the balance active clean-up material chosen from the group consisting of the alkali metals, the alkaline earth metals, the rare earth metals, and alloys thereof containing at least about 15% of the said metals; the copper being physically separable from the active material and being present in sufficient amount to impart a reddish color to the clean-up agent.

5. A reddish-colored clean-up agent comprising a coherent aggregate of comminuted copper 10 and comminuted silver-colored active clean-up material, the copper forming about 25% to 50% of the said aggregate and being physically separable from the active clean-up material.

6. A getter assembly comprising a thin piece 15 of substantially silver-colored metal provided with a depression, and a reddish-colored clean-up agent containing copper and silver-colored active clean-up material firmly secured in the depression, the copper forming about 25% to 20 50% of the said agent and being physically separable from the said active clean-up material.

7. A getter assembly comprising a thin piece 25 of substantially silver-colored metal provided with a depression, and firmly secured in the depression, a reddish-colored clean-up agent composed of copper and an alloy of magnesium with an alkaline earth metal, the copper forming about 25% to 50% of said agent and being physically separable from said alloy.

JOHN D. McQUADE.